

## UNITED STATES PATENT OFFICE

2,443,322

## EMULSIFICATION OF COAL TAR PITCH

John Alexander Montgomerie, Cambuslang, and Peter Kennedy Archibald, Bearsden, Scotland, and Leonard Charles Bradshaw, Langley, England, assignors to International Bitumen Emulsions Limited, Slough, England, a corporation of Great Britain

No Drawing. Application February 6, 1945, Serial No. 576,512. In Great Britain December 2, 1943.

2 Claims. (Cl. 252—311.5)

1

This invention relates to the controlled preparation of aqueous emulsions of coal tar pitch.

Heretofore it has not been considered to be commercially practicable to emulsify unselected coal tar pitch having a melting point above 50° C., and having a working fluidity only at a temperature above 100° C., notwithstanding that such coal tar pitch has a wide field of application in the coating or impregnation of paper and paper board.

In seeking to emulsify coal tar pitch from different sources by the process described in the specification of British Patent No. 462,111, we have occasionally obtained irregular results, due to variations in the chemical and physical properties of such pitches even when of substantially the same melting point and comparable fluidity.

As the result of experimental research we have now found that the irregular results mentioned above can be largely eliminated by using natural asphalt, such as Trinidad asphalt, as an assistant emulsifier in the emulsification of coal tar pitch, it may be in conjunction with a proportion of fatty acid pitch or fatty acid, and dispersing the blend in a hot dilute aqueous solution of an alkali, preferably a fixed alkali, employing as an additional assistant emulsifier a protein compound, with or without the presence of an organic salt or salts, for example, sodium oleate, with or without the presence of a colloidal clay such as bentonite.

For the purpose of our invention the Trinidad asphalt may be blended (a) with the coal tar pitch before the addition of fatty acid or fatty acid pitch, or (b) with fatty acid or fatty acid pitch before its addition to the coal tar pitch.

## Example

1400 lbs. of a composition of coal tar pitch, Trinidad asphalt and linseed acid oil in the proportions by weight, respectively, of 100:10:7.5 are emulsified by stirring into 30 gallons of boiling water, to which have been added 30 lbs. of dry bentonite, 10 lbs. of caustic soda and 100 lbs. of dry casein. 100 gallons of additional water and 20 lbs. of cresylic acid are added during or after the formation of the emulsion.

The linseed acid oil referred to in the preceding examples and in the appended claims, functions as an assistant emulsifier. It is a by-product of the alkali refining of linseed oil. When linseed oil is treated with hot aqueous alkali, the free fatty acids present in the linseed oil are saponi-

fied and are dissolved in the aqueous medium in which the alkali was dissolved. On standing, the aqueous and oleaginous phases resolve into lower and upper layers, respectively. The aqueous phase after being separated is acidified with sulfuric acid to precipitate the free fatty acids and two layers again form. The oleaginous layer is linseed acid oil, the approximate composition of which is:

|                                                                      | Per cent |
|----------------------------------------------------------------------|----------|
| Linseed-oil-free fatty acids (contained in the original linseed oil) | 50       |
| Entrained linseed oil                                                | 40       |
| Mucilage and water                                                   | 10       |

## We claim:

1. The process of producing an aqueous emulsion of a coal tar pitch having a melting point above 50° C. and a working fluidity only at a temperature above 100° C., which comprises blending the coal tar pitch with an assistant emulsifier comprising Trinidad asphalt and "linseed acid oil," and dispersing the blend of coal tar pitch, Trinidad asphalt and "linseed acid oil" in a hot dilute aqueous alkaline solution.
2. The process of producing an aqueous emulsion as defined by claim 1, in which 10 parts by weight of Trinidad asphalt and 7.5 parts by weight of "linseed acid oil" are blended with each 100 parts by weight of coal tar pitch.

JOHN ALEXANDER MONTGOMERIE.

PETER KENNEDY ARCHIBALD.

LEONARD CHARLES BRADSHAW.

## REFERENCES CITED

The following references are of record in the file of this patent:

## UNITED STATES PATENTS

| Number    | Name                  | Date          |
|-----------|-----------------------|---------------|
| 2,190,604 | Montgomerie et al. -- | Feb. 13, 1940 |
| 1,734,437 | Kirschbraum -----     | Nov. 5, 1929  |
| 1,725,648 | Kirschbraum -----     | Aug. 20, 1929 |

## FOREIGN PATENTS

| Number  | Country             | Date          |
|---------|---------------------|---------------|
| 462,111 | Great Britain ----- | Mar. 2, 1937  |
| 421,269 | Great Britain ----- | Dec. 6, 1934  |
| 332,591 | Great Britain ----- | July 22, 1930 |
| 28,178  | Great Britain ----- | 1910          |
| 670,870 | France -----        | Aug. 26, 1929 |
| 665,060 | France -----        | Apr. 30, 1929 |
| 134,983 | Austria -----       | Oct. 25, 1933 |